

- [54] **PROCESS FOR PRODUCING DURABLE PRESS TEXTILES**
- [75] Inventors: **Richard P. Barber; Glen R. Moses**, both of Mooresville, N.C.
- [73] Assignee: **Burlington Industries, Inc.**, Greensboro, N.C.
- [22] Filed: **June 11, 1971**
- [21] Appl. No.: **152,428**
- [52] U.S. Cl. .... **38/144**, 8/116.3, 8/115.6, 117/11, 117/139.4, 117/143 A, 117/161 UT
- [51] Int. Cl. .... **D06m 13/54**, D06m 13/40
- [58] Field of Search ..... 117/139.4, 139.5 A, 117/143 A, 11, 161 UT, 10; 8/115.6, 116.3; 260/851, 856; 38/144

[56] **References Cited**

UNITED STATES PATENTS

- 3,446,777 5/1969 Emmons..... 117/142 X

|           |         |                     |             |
|-----------|---------|---------------------|-------------|
| 2,950,553 | 8/1960  | Hurwitz .....       | 117/143 A   |
| 3,220,869 | 11/1965 | Ruemens et al. .... | 117/139.4 X |
| 3,096,524 | 7/1963  | Mizell.....         | 117/139.4 X |
| 2,623,031 | 12/1952 | Snyder .....        | 260/75 P    |
| 3,186,954 | 6/1965  | Hushebeck .....     | 117/139.4 X |
| 3,159,562 | 11/1964 | Kine et al. .....   | 161/170     |

*Primary Examiner*—William D. Martin  
*Assistant Examiner*—Theodore G. Davis  
*Attorney*—Cushman, Darby & Cushman

[57] **ABSTRACT**

Disclosed herein is a process for producing a durable press cellulosic textile fabric comprising to the fabric applying an aqueous mixture of a thermosetting durable press textile reactant, and a crosslinking acrylic polymer, a crosslinking catalyst, making the fabric into a garment or article and subsequently pressing and curing said mixture on the article.

8 Claims, No Drawings

## PROCESS FOR PRODUCING DURABLE PRESS TEXTILES

The preparation of durable press textiles comprising cellulosic fibers, e.g., knitted or woven fabric made up of blends of cotton and polyester, is now well known. Procedures for preparing such textiles involve applying an aqueous composition containing a durable press reactant to cellulosic fabric, drying, pressing and curing. When a durable press garment is to be made, the dried fabric is usually cut and sewn into the desired form, e.g., pants, and then pressed and cured. Pressing and curing may be carried out simultaneously at relatively high temperatures (see U. S. Pat. No. 2,950,553) although the more widely practiced technique is to press the garment at a somewhat lower temperature (such as 300°-335°F.) using, for example, a hot head press, followed by a separate baking or curing operation in an oven at higher temperatures (e.g., 350°-375°F.).

A number of variations in the above procedures, or alternatives thereto, are also known in the art. For example, U. S. Pat. No. 3,341,955 describes the preparation of durable press garments from 100 percent cotton fabrics by padding the fabric with an aqueous durable press reactant finish, drying and curing. Thereafter, when a garment with a permanent crease is to be made, the area where the crease is desired is treated with acid catalyst and pressed at high temperature (350°F. or above).

A further alternative is also described in U.S. Pat. No. 3,341,955 for use when the fabric comprises a blend of cotton and thermoplastic fibers, such as polyester. In that embodiment, the fabric, after application of the durable press finish, and drying, is formed into a garment and pressed, sufficient heat being applied during pressing to soften and set the thermoplastic component in the desired shape. Temperatures in the order of 350° to 500°F., depending on the softening point of the thermoplastic fibers, are utilized for the press-setting operation.

While the above procedures give useful durable press effects, several disadvantages are also presented thereby. For example, oven baking a fabric composed entirely of cotton causes a significant deterioration of the cotton with resultant loss in such physical properties as tensile strength, tear strength and abrasion resistance. Blending of the cotton with polyester or the like brings about some improvement in physical properties but the cellulosic component in such blends is still undesirably degraded. This degradation shows up in a number of ways, e.g. by reduced abrasion resistance, and is especially noticeable after washing cotton/polyester durable press fabrics, the degraded cotton being washed out, along with hand builders or softeners attached thereto, so that the fabric becomes sleepy or thin.

The procedures which involve oven baking also have economic disadvantages, not only in the cost and maintenance of the ovens, but in the relatively long time required (10-15 minutes) to accomplish the desired cure. The curing time also has an undesirable effect on fabric color, e.g., hue or cast may be changed and/or whites may be caused to yellow. The simultaneous press/cure procedures are generally free from these problems but they suffer from other disadvantages and,

in general, do not give as good a durable press effect as the procedures involving oven curing.

The principal object of the present invention is to provide durable press textiles and procedures for making the same whereby the above-noted problems with prior procedures are eliminated or substantially reduced. A further object is to provide cellulosic fabrics which have, in addition to an outstanding durable press, other improved physical and aesthetic properties.

Still another object of the invention is to provide a process for obtaining durable press effects on cellulosic textiles using less severe press/cure conditions than previously utilized, with resultant improvement in the overall properties of the product. A more specific object is to provide a durable press finish and process whereby pressing and curing may be effectively carried out simultaneously on the press using lower temperatures and shorter times than normally considered feasible.

Broadly stated, the objects of the invention are realized by treating the fabric with an aqueous formulation of one or more low temperature crosslinking film-forming acrylic polymers, a durable press thermosetting fiber-reactive resin and a curing or cross-linking agent; drying, pressing and curing, the fabric being formed into a garment or other article (e.g., sheets) before the pressing and curing. Preferably a mixture of crosslinking acrylic polymers is used and/or the formulation includes a heat curable or crosslinking elastomer hand builder as described below.

As noted earlier herein, an advantage of the invention is that pressing and curing can be carried out simultaneously using relatively moderate times and temperatures with resultant improvement in the properties of the treated fabric. For example, fabric processed according to the invention can be press-cured on a hot head press at temperatures not exceeding 345°F., typically in the range of 300°F. to 345°F. and in some instances even lower (280°-290°F.) using normal pressing times such as 15 seconds (usually 5 seconds steam, 5 seconds vacuum and 5 seconds dry) to give highly durable creases and wash and wear properties in the pressed fabric. Additionally, aesthetic properties such as hand, feel and color and physical characteristics, e.g., tensile strength, tear and abrasion resistance, are not undesirably affected.

The success of the invention is due, at least in large measure, to the use of the low temperature crosslinking acrylic polymer in combination with the durable press fiber reactant and curing agent. It is not understood how or why the indicated components function to give the stated results but it is apparent, in any event, that this combination must be used to obtain the overall results of the invention. It appears that the indicated components somehow work together in a synergistic fashion to give the results indicated since durable press properties, for example, exceed those which would be expected from the normal additive effect of the individual components.

The acrylic polymer used herein may be defined as a copolymer of a lower alkyl ester of acrylic acid or methacrylic acid, or like monoethyleneically unsaturated compound, with another monomer copolymerizable therewith and additionally including

one or more functional groups capable of undergoing crosslinking, e.g., carboxy or hydroxy groups. Preferably the polymer is a water-insoluble or water-dispersible addition copolymer of

1. from 0.5 to 99.5 percent by weight of a guanamine compound of the formula



where R is an alkenyl group having 3 to 9 carbon atoms and a terminal group of the formula



R<sup>0</sup> is H, CH<sub>2</sub>OH, or CH<sub>2</sub>OR'' wherein R'' is the hydrocarbon residue of a saturated alcohol R''OH having one to eight carbon atoms,

R' is H, CH<sub>2</sub>OH, or CH<sub>2</sub>OR''

R<sup>2</sup> is H, CH<sub>2</sub>OH, or CH<sub>2</sub>OR'', and

R<sup>3</sup> is H, CH<sub>2</sub>OH, or CH<sub>2</sub>OR'', and

2. from 99.5 to 0.5 percent by weight of one or more monomers selected from acrylic acid, methacrylic acid, the nitriles thereof, the esters thereof with a saturated aliphatic alcohol having one to 18 carbon atoms, acrylamide, methacrylamide, the N-methylol derivatives of these amides, itaconic acid, vinyl acetate, vinyl chloride, styrene, and o-, m-, and p-vinyltoluene. Copolymers of this type are described in U. S. Pat. No. 3,446,777 and any of the low temperature crosslinking acrylic polymers described therein may be used for present purposes. Preferred comonomer proportions comprise about 0.5 to 30 percent by weight of monomer (1) and the balance essentially one or more of comonomers (2). Such polymers may have molecular weights in the order of 1,000 to 1,000,000 and are available in latex or emulsion form. A particularly preferred low temperature crosslinking acrylic copolymer for use herein is the product of Example 10 of U.S. Pat. No. 3,446,777 but using butyl acrylate instead of the ethyl acrylate referred to therein (i.e. the copolymer of butyl acrylate and methylolated-4-pentenoguanamine) with the pH modified from 5.4 to 9.0 by addition of ammonia to improve emulsion stability. Similar copolymers of methylolated-4-pentenoguanamine with, for example, ethyl acrylate or other lower alkyl acrylates, may also be used.

It is particularly advantageous to utilize a mixture of two different low temperature crosslinking acrylic polymers for present purposes and an especially useful embodiment of the invention contemplates using a mixture of the low temperature crosslinking acrylic copolymer of a lower alkyl acrylate and methylolated-4-pentenoguanamine as described above together with the water insoluble, water-dispersible low temperature self-crosslinking acrylic copolymers of a lower alkyl acrylate (e.g., ethyl or butyl acrylate) and an N-methylolacrylamide as described in U.S. Pat. No. 3,157,562, e.g., the copolymer of 90-99 percent lower alkyl acrylate, 1-10 percent N-methylolacrylamide and optionally from 0-3 percent acrylamide.

According to the invention it is also advantageous to include in the durable press formulation a curable elastomer or like hand builder. The elastomer component, if used, is most desirably a heat curable polyester elastomer hand builder although other elastomers may be used. The term "elastomer" as used herein has the meaning given by The American Society for Testing Materials as described in the Encyclopedia of Chemical Technology, 2nd Edition, Volume 7, page 676. This is "a material that is capable of recovery from large deformations quickly and forcibly and can be . . . modified to a state in which it is essentially insoluble (but can swell) in boiling solvents such as benzene, methyl ethyl ketone and the ethanol-toluene azeotrope. A rubber in its modified state, free of diluents, retracts within one minute to less than 1.5 times its original length after being stretched at room temperature (20-27° before release.)"

A wide variety of elastomers may be used for present purposes, although they are primarily grouped into several recognized categories. As indicated, the preferred category comprises the polyester elastomers including Paraplex rubbers (see Industrial and Engineering Chemistry, Volume 39, page 1090 (1947), Norepal polyester rubbers derived from ethylene glycol and dimeric soya beam fatty acids, copolymer of terephthalic acid and acyclic dicarboxylic acid and a glycol (see U.S. Pat. Nos. 2,623,033 and 2,623,031), all polyesters linked together by diisocyanates, for example, polyethylene adipate linked by 1,5-naphthalene diisocyanate (see "Polyesters and their Applications," by Bjorksten et al., 1956, page 226). These are related to polyurethane elastomers which are cross-linked by diisocyanates.

Other heat-curable elastomers which may be used herein, in lieu of or in addition to a polyester elastomer, include, for example, acrylic elastomers, olefin polymers and the homopolymers and copolymers of dienes such as butadiene, isoprene and chloroprene. The acrylic elastomers are addition type polymers and copolymers which contain a predominant amount of an acrylic acid ester with an alcohol having two or more carbon atoms such as ethyl acrylate or butyl acrylate. These may be crosslinked through the hydrogen atom adjacent the carboxyl group of the acrylic acid moiety by means of a peroxide or by including a small amount (e.g., about 5 percent) of functional groups such as olefinic groups, halogen, carboxyl and cyano.

The olefin elastomers include ethylene-propylene rubber and butyl rubber. Ethylene-propylene rubber typically contains 40-70 percent ethylene, the balance being propylene. Butyl rubber typically comprises 0.5-2.5 percent molar isoprene, balance isobutene. Polyvinyl alcohol, polyvinyl acetate and the like may also be included in the formulation along with conventional types of softeners, surfactants, etc.

As the durable press reactant component of the present finish, any of the conventional durable press, reactant resins may be used. Typically, the resin is a water-soluble precondensate of formaldehyde with such amino compounds as urea, thiourea, cyclic ethylene ureas (e.g., dimethylol cyclic ethylene urea or dimethylol dihydroxy cyclic ethylene urea), melamine, ethyl carbamate, urons, triazones and triazines or mix-

tures thereof. Blocked isocyanates may also be effectively used.

Suitable crosslinking or curing catalysts for use herein include, without being limited thereto, magnesium chloride or nitrate or zinc chloride or nitrate; various amine hydrochlorides such as 2-amino-2-methyl-1-propanol hydrochloride, or triethanol-amine hydrochloride; and ammonium salts such as ammonium chloride, tartrate, citrate, formate, oxalate, nitrate or ammonium ethyl phosphate or ammonium dihydrogen phosphate or the like. These catalysts may be combined, e.g., zinc nitrate and ammonium chloride may be used together, and/or catalyst modifiers may be included as necessary to achieve desired effects, e.g., to increase or decrease catalyst activity. It is particularly useful to employ citric acid in conjunction with zinc chloride, or other catalyst since the citric acid makes it possible to effectively utilize even lower pressing temperatures, e.g., 280°F., as described later herein.

It may also be helpful in some cases to include additives such as boric acid, the latter being useful to avoid any tendency of the pressed fabric to yellow in the event of an after-curing operation.

Typically, the finish of the invention will comprise, on a weight basis, from 3-20 percent of the low temperature cross-linking acrylic polymer or mixtures thereof, 0-15 percent, preferably 5-10 percent heat curable elastomer; 3-25 percent durable press resin; and 0.1-7 percent catalyst, balance water. Additionally, the finish may include from 0 to 5 percent (usually 0.2-2 percent) surfactant, and from 0-10 percent of other conventional durable press components such as extenders, softeners or the like.

The finish is applied to the fabric in any convenient fashion, e.g., by dipping or spraying but preferably by padding. The amount of the finish applied can be widely varied and is dependent on such factors as the nature and construction of the fabric, its intended use, etc. Usually, however, wet pickup will fall in the range of 30-75 percent by weight of the fabric. The thus-treated fabric is then dried, usually at 190-220°F. for 1-5 minutes, to a moisture content in the order of 5-10 percent by weight.

The dried fabric is then cut into the desired shape, sewn into a garment or other article and pressed on a hot head press or the equivalent. Typical pressing conditions comprise pressing on the hot head press at 300°-345°F. for up to 15 seconds or so. Curing or baking in an oven is not necessary since, with the finish of the invention, durable press effects are obtained by pressing only. However, if desired, the pressed article may be baked under proper conditions without serious disadvantages. If, as in some cases, it is desired to produce an excellent wash and wear fabric, then fabrics treated with this finish can be precured or cured in the finishing plant at 280°-345°F. for 30 to 180 seconds.

The invention is illustrated, but not limited, by the following examples wherein percentages are by weight unless otherwise indicated:

#### EXAMPLE 1

The following formulation was prepared in warm water (e.g., 80°-100°F.) by adding the components in the order listed to sufficient water to give the indicated percent concentration.

0.10 percent alkylaryl polyester alcohol (Triton X-155)

5 5.00 percent glyoxal resin (1)

5.00 percent polyester resin (2)

5.00 percent fast curing acrylic emulsion (3)

3.00 percent acrylic ester emulsion (4)

3.00 percent cationic quaternary ammonium softener (5)

3.00 percent zinc chloride solution, 50% in water

10 The above components (1) - (5) may be more fully defined as follows:

Component (1): N,N-dimethylol dihydroxyethylene urea, 50 percent solution in water;

15 Component (2): a polyester of phthalic anhydride, polyethylene glycol and glycerides of hydrogenated fatty acids (commercially available as "Discol 716");

Component (3): the product of Example 10 of U.S. Pat. No. 3,446,777 with the substitution of butyl acrylate for the ethyl acrylate used in Example 10 and with adjustment of the pH of the emulsion to 9 by addition of ammonia to stabilize the emulsion;

20 Component (4): an aqueous emulsion of 75/25 ethyl acrylate/vinyl acetate copolymer, solids content 40 percent (commercially available as "Wicaset P.E.P.");

Component (5): crude dimethyldistearylammonium hydrogen sulfate, the stearyl groups being predominant in a mixture of higher alkyl radicals derived from hydrogenated tallow.

25 30 The following fabrics (A) - (D) were padded through the above formulation followed by drying for 1½ minutes at 300°F.

A few days later the above fabrics were pressed on a hot head press for 5 seconds steam, 5 seconds vacuum, 35 5 seconds dry at 345°F. and 80 pounds air (9,000 psi in head). The thus pressed fabrics were then home laundered five times with tumble drying after each laundering. The laundered fabrics were then checked for wash/wear and crease appearance and evaluated using a grade rating of from 1-5, values of 1-3 being considered unacceptable and 5 representing the optimum. The results obtained are shown below.

| 45                           | Fabric | Wash/Wear Appearance | Crease Appearance |
|------------------------------|--------|----------------------|-------------------|
| (A) Polyester/cotton (50/50) | 3.6    | 5.0                  |                   |
| (B) Polyester/cotton (50/50) | 4.0    | 5.0                  |                   |
| (C) Polyester/cotton (50/50) | 4.3    | 5.0                  |                   |
| (D) Polyester/rayon (50/50)  | 4.6    | 5.0                  |                   |

50 As will be evident, specimens (A) - (D) demonstrated effective durable press and wash/wear properties notwithstanding the fact that the specimens were only pressed on the hot head press to obtain these properties. The laundered specimens were also characterized by outstanding physical and aesthetic properties, e.g., abrasion resistance, tensile and tear strength, hand, feel and the like.

#### EXAMPLE 2

55 Example 1 was repeated except that the formulation was changed to include 20 percent of the glyoxal resin (1), rather than 5 percent; and the polyester resin (2) and acrylic ester emulsion (4) were replaced by 5 percent self-crosslinking acrylic emulsion (6), namely, an aqueous emulsion of a copolymer of butyl acrylate and an N-methylolacrylamide per U.S. Pat. No. 3,157,562.

Three fabrics (E, F and G) of the same construction as used in Example 1 were processed in similar fashion with the thus modified formulation and evaluated for wash/ wear appearance, crease appearance and total shrinkage with the following results:

| Fabric                       | Wash/Wear Appearance | Crease Appearance | Total Shrinkage |
|------------------------------|----------------------|-------------------|-----------------|
| (E) Polyester/cotton (50/50) | 4.0                  | 5.0               | 1.94 x 1.39     |
| (F) Polyester/cotton (50/50) | 4.0                  | 5.0               | 2.67 x 1.19     |
| (G) Polyester/cotton (50/50) | 3.6                  | 5.0               | 2.58 x 1.11     |

The indicated wash/wear, crease and shrinkage values are satisfactorily within acceptable limits for these properties.

### EXAMPLE 3

Example 2 was repeated except that the amount of zinc chloride catalyst was increased to 6 percent and the amount of self-crosslinking acrylic emulsion was reduced to 3 percent with the following results indicating acceptable wash/wear, crease and shrinkage properties.

| Fabric                   | Wash/Wear Appearance | Crease Appearance | Total Shrinkage |
|--------------------------|----------------------|-------------------|-----------------|
| Polyester/cotton (50/50) | 4.0                  | 5.0               | 2.50 x .92      |
| Polyester/cotton (50/50) | 4.3                  | 5.0               | 2.02 x .36      |
| Polyester/cotton (50/50) | 4.3                  | 5.0               | 2.78 x .72      |

### EXAMPLE 4

Example 1 was repeated using the following aqueous formulation:

- 0.10 percent alkylaryl polyether alcohol (Triton X-155)
- 20.0 percent glyoxal resin (1)
- 5.00 percent fast curing acrylic emulsion (3)
- 5.00 percent polyester resin (7)
- 3.00 quaternary ammonium softener (5)
- 3.00 percent zinc chloride catalyst solution, 50% in water
- 3.00 percent ammonium chloride solution, 25% in water
- 0.5 percent boric acid

The polyester resin (7) was Aerotex Resin DHB (American Cyanamid), described as a 57 percent active, self-emulsifying cross-linkable polyester resin in xylene, used for durable hand building.

The following results were obtained in fabric specimens as indicated:

| Fabric                   | Tensile Strength lbs. | Wash/Wear Appearance | Crease Appearance |
|--------------------------|-----------------------|----------------------|-------------------|
| Polyester/cotton (50/50) | 117 x 86              | 4.3                  | 5.0               |
| Polyester/cotton (50/50) | 101 x 73              | 4.0                  | 5.0               |
| 100% cotton              | 67 x 57               | 4.0                  | 4.0               |

A further embodiment of the invention contemplates the use of catalyst combinations which will permit the application of the desired durable press effects at even lower pressing temperatures than those indicated above. It is possible, for example, by using an aqueous

solution comprising zinc chloride and 1-6 percent citric acid as the catalyst to so lower the temperature at which a durable press can be imparted (e.g., 260°-300°F. for 10-30 seconds) that the durable press can be accomplished at home using a hand steam iron or a hot flat iron. In other words, the use of a solution of 1-6 percent citric acid and, for example, zinc chloride or the like in conventional amounts (e.g., from 1 to 6 percent) makes it possible to reduce the effective pressing or curing temperature of the system by from 20°-30°F. using press times in the order of 10-30 seconds, advantageously 15-20 seconds. The presence of the citric acid also tends to reduce the amount of total shrinkage in the processed fabric (i.e., heat shrinkage and washed shrinkage). In other words, the citric acid seems to stabilize the fabric without the need to sanforize. Apparently the citric acid and zinc chloride or other catalyst somehow coact to initiate partial reaction with one or more of the resinous components of the finish during the initial drying operation, after application of the finish to bring about the desired results although the actual mechanism is not understood.

The advantages of using citric acid in the catalyst system are shown by the following additional examples:

### EXAMPLE 5

A formulation was prepared as in Example 1 using the following components in the indicated amounts:

- 0.10 percent alkylaryl polyester alcohol (Triton X-155)
  - 0.50 percent nonylphenoxy poly(ethyleneoxy)ethanol (Igepal CO-897)
  - 20.00 percent glyoxal resin (1)
  - 7.50 percent fast curing acrylic emulsion (3)
  - 7.50 percent self crosslinking acrylic emulsion (6)
  - 2.00 percent tall oil ester softener
  - 6.00 percent zinc chloride solution, 50 percent in water
  - 6.00 percent citric acid solution, 40 percent in water
- Polyester/cotton (50/50) fabrics as in Example 1 were padded through the above formulation, dried at 300°F. for 1½ minutes and subsequently pressed. One set of fabrics was pressed on the hot head press at 325°F. for 15 seconds, another set was pressed at 290°F. for 15 seconds, with the following crease values and wash/wear results, after five home launderings.

| Fabric Weight<br>Ozs./Sq.Yd. | Pressed at 325°F.<br>15 seconds |                      | Pressed at 290°F.<br>15 seconds |                      |
|------------------------------|---------------------------------|----------------------|---------------------------------|----------------------|
|                              | Crease                          | Wash/Wear Appearance | Crease                          | Wash/Wear Appearance |
| 5.40                         | 5.0                             | 4.8                  | 5.0                             | 4.8                  |
| 6.50                         | 5.0                             | 4.8                  | 5.0                             | 4.8                  |
| 8.50                         | 5.0                             | 4.8                  | 5.0                             | 4.8                  |

### EXAMPLE 6

Example 5 was repeated except that the amount of citric acid used was reduced to 4 percent and the fabrics tested were as shown below with the following results:

| Fabric Weight | Fabric Blend          | Pressed at 290°F.<br>15 seconds |                         | Total Shrinkage<br>(Heat/Wash) |
|---------------|-----------------------|---------------------------------|-------------------------|--------------------------------|
|               |                       | Crease<br>Appearance            | Wash/Wear<br>Appearance |                                |
| 6.30          | Polyester/rayon 65/35 | 5.0                             | 4.6                     | 1.83 x 0.93                    |

|     |                           |     |     |                |
|-----|---------------------------|-----|-----|----------------|
| 6.0 | Polyester/cotton<br>50/50 | 5.0 | 4.6 | 1.75 x<br>0.67 |
|-----|---------------------------|-----|-----|----------------|

The above results show that the exemplified process, using citric acid as a catalyst component, gives outstanding crease and wash/wear properties and dimensional stability using lower than normal pressing temperatures.

#### EXAMPLE 7

The following formulations were prepared in warm water by adding the components in the order listed.

| Formula I | Formula II |                                                                    |
|-----------|------------|--------------------------------------------------------------------|
| 0.10%     | 0.10%      | alkylaryl polyether alcohol<br>(Triton X-155)                      |
| 0.50%     | 0.50%      | nonylphenoxy poly(ethyleneoxy)<br>ethanol (Igepal CO-897)          |
| 20.00%    | 20.00%     | glyoxal resin (1)                                                  |
| 7.50%     | 7.50%      | fast curing acrylic emulsion (3)                                   |
| 7.50%     | 7.50%      | self crosslinking acrylic emulsion<br>(6)                          |
| 3.00%     | 3.00%      | high density polyethylene, 29%<br>aqueous emulsion (Aqualene<br>N) |
| 6.00%     | 3.00%      | zinc chloride solution, 60% in<br>water                            |
|           | 3.00%      | citric acid solution, 40% in water                                 |

Two light weight fabrics (50/50 polyester/cotton blend and a white 100 percent cotton) were treated with the above formulas. Wet pickup was 65-75 percent, fabrics dried for 1 1/2 minutes at 300°F. Pant legs were made and were creased and pressed with a hand steam iron for approximately 30 seconds on each side. The following data show wash/wear and crease appearance after five home launderings and the tensile strength and abrasion properties.

| Tensile-Warp<br>(Pounds)           | Hand Steam Iron<br>100% Cotton |         | Hand Steam Iron<br>50/50<br>Polyester/Cotton |         | Experiment<br>No. 1<br>No. 2<br>No. 3<br>No. 4 | Crease<br>Appearance<br>5.0<br>5.0<br>5.0<br>5.0 | Wash/Wear<br>Appearance<br>4.0<br>5.0<br>5.0<br>5.0 |
|------------------------------------|--------------------------------|---------|----------------------------------------------|---------|------------------------------------------------|--------------------------------------------------|-----------------------------------------------------|
|                                    | Formula                        | Formula | Formula                                      | Formula |                                                |                                                  |                                                     |
|                                    | I                              | II      | I                                            | II      |                                                |                                                  |                                                     |
| Filling                            | 50                             | 50      | 39                                           | 46      |                                                |                                                  |                                                     |
| Crease Appearance                  | 5.0                            | 5.0     | 5.0                                          | 5.0     |                                                |                                                  |                                                     |
| Wash/Wear Appearance               | 4.0                            | 4.0     | 4.0                                          | 4.0     |                                                |                                                  |                                                     |
| Abrasion                           | 429                            | 492     | 2000+                                        | 2000+   |                                                |                                                  |                                                     |
| Untreated Tensile-Warp<br>(Pounds) | 65                             | 65      | 65                                           | 65      |                                                |                                                  |                                                     |
| Filling                            | 59                             | 59      | 38                                           | 38      |                                                |                                                  |                                                     |

#### EXAMPLE 8

The following formulation was prepared in warm water by adding the components in the order listed.

0.10 percent alkylaryl polyether alcohol (Triton X-155)  
0.50 percent nonylphenoxy poly(ethyleneoxy)ethanol (Igepal CO-897)  
20.00 percent glyoxal resin (1)  
7.50 percent fast curing acrylic emulsion (3)  
5.00 percent acrylic latex (Hycar 2679)  
2.00 high density polyethylene, 29 percent aqueous emulsion (Aqualene N)  
6.00 percent zinc chloride solution, 60 percent in water  
4.00 percent citric acid solution, 40 percent in water

Approximately 18,000 yards of a 50/50 polyester/cotton fabric were treated by padding the above formula, tenter drying followed by running the fabric over the palmer unit of a sanforizer.

5 Several samples were taken throughout the run. Pant legs were made and pressed for 15 seconds at 280°F. with 70 pounds of air on pressing head.

The following data is the average of these several sample representing 18,000 yards.

| 10 | Fabric Weight<br>Ozs./Sq.Yd. | Tensile<br>(Grab<br>lbs.) | Crease<br>Appearance*<br>5.0 | Wash/Wear<br>Appearance*<br>4.3 | %Shrinkage<br>2.15 x<br>0.73 |
|----|------------------------------|---------------------------|------------------------------|---------------------------------|------------------------------|
|    | 15 7.42                      | 174 x 109                 |                              |                                 |                              |

\*as measured after 5 home launderings

#### EXAMPLE 9

20 The following formulation was prepared in warm water by adding the components in the order listed.

0.10 percent alkylaryl polyether alcohol (Triton X-155)

0.50 percent nonylphenoxy poly(ethyleneoxy)ethanol (Igepal CO-897)

20.00 percent glyoxal resin (1)

7.50 percent fast curing acrylic emulsion (3)

7.50 percent self crosslinking acrylic emulsion (6)

2.00 percent tall oil ester softener

30 6.00 percent zinc chloride solution, 60 percent in water

-%\* citric acid solution, 40 percent in water

\*varying amounts of citric acid as below

The fabric used was a 50/50 polyester/cotton blend.

35 Fabric specimens were pressed at 290°F. for 15 seconds. Washed five times.

| 40 | Hand Steam Iron<br>100% Cotton | Hand Steam Iron<br>50/50<br>Polyester/Cotton | Experiment<br>No. 1<br>No. 2<br>No. 3<br>No. 4 | Crease<br>Appearance<br>5.0<br>5.0<br>5.0<br>5.0 | Wash/Wear<br>Appearance<br>4.0<br>5.0<br>5.0<br>5.0 |  |
|----|--------------------------------|----------------------------------------------|------------------------------------------------|--------------------------------------------------|-----------------------------------------------------|--|
|    | Formula<br>I<br>54             | Formula<br>II<br>55                          | Formula<br>I<br>62                             | Formula<br>II<br>61                              |                                                     |  |

45 As can be seen from the above data acceptable crease and wash and wear appearance were obtained with and without the use of citric acid by pressing the treated fabric at 280°F. although wash and wear appearance was maximized with the addition of 1 percent or more of citric acid.

50 It will be appreciated that various modifications may be made in the invention described herein. Hence the scope of the invention is defined in the following claims wherein:

We claim:

55 1. A process for providing a durable press on a cellulosic textile garment or other article which comprises applying to cellulosic textile fabric a finish comprising an aqueous mixture of, on a weight basis, 3-25 percent of a thermosetting durable press textile reactant, 3-20

60 percent of at least one low temperature crosslinking acrylic polymer, and 0.1-7 percent of a crosslinking catalyst, drying, cutting said fabric into pieces and sewing the same together into said garment or article and pressing the resulting article in the desired shape and simultaneously curing the finish so as to obtain said durable press, the pressing and curing being carried out at a temperature not in excess of about 345°F.

65

2. The process of claim 1 wherein the cross-linking acrylic polymer comprises the copolymer of a lower alkyl acrylate and methyololated-4-pentenoguanamine.

3. The process of claim 1 wherein the pressed and cured textile article is subsequently further cured.

4. The process of claim 1 wherein the catalyst is a mixture of zinc chloride and citric acid and the textile is pressed at 260°-280°F.

5. A durable press textile article obtained by the process of claim 1.

6. The process of claim 2 wherein a mixture of cross-linking acrylic polymers is used comprising the copolymer of a lower alkyl acrylate and methyololated-4-pentenoguanamine and the copolymer of a lower alkyl acrylate and an N-methyololacrylamide.

7. The process of claim 2 wherein the mixture also includes a film-forming heat curable elastomer.

8. The process of claim 7 wherein the elastomer is a polyester elastomer.

\* \* \* \* \*